

## UNITED STATES PATENT OFFICE

2,072,824

## METHOD OF MAKING CASTOR OIL SOAP

Oney P. Puryear, Beacon, N. Y., assignor to The Texas Company, New York, N. Y., a corporation of Delaware

No Drawing. Application May 7, 1934,  
Serial No. 724,463

3 Claims.

(Cl. 87—5)

This invention relates to lubricants and particularly to lubricants containing a soluble castor oil ingredient.

An object of the invention is to produce an improved castor oil product which is soluble in mineral oil.

A further object of the invention is to form a castor oil soap which is soluble in mineral lubricating oils.

Another object of the invention is to provide a simple and practical method of preparing lubricants containing a soluble castor oil soap ingredient.

Another object of the invention is to produce an improved grease containing a soluble castor oil soap.

Castor oil is ordinarily insoluble in petroleum oils and several methods have been devised for rendering it soluble therein. The prior methods include distillation with or without the addition of a carrier oil whereby about 4-5% of oxygen-containing materials are removed. The resulting product, while soluble, is often thick and gummy and has an objectionable odor and color. Another method has consisted in using a solvent aid or blending agent which is mutually soluble in castor oil and mineral oils but these third ingredients are often undesirable.

Soluble metallic soaps of castor oil have also been made heretofore but such has been done by first producing a soluble castor oil product and then forming the metallic soap of the soluble product. The soaps made according to prior methods, however, have in general the disadvantages of the soluble castor oil from which they are made.

I have found that an improved soluble castor oil soap may be made easily and practically by saponifying ordinary castor oil to form a soap mixture which is normally insoluble in mineral oil and then heating this mixture to sufficient temperature to vaporize the products which render the castor oil insoluble. The product so obtained is miscible with mineral oils and serves as a convenient ingredient for incorporation into greases. If desired, the castor oil in a soluble form may be recovered by well known means from the soap to obtain a mineral oil-soluble castor oil product.

In accordance with the invention, the castor oil to be treated is put into a suitable heating vessel, such as a grease kettle, and alkali slowly added with stirring. The castor oil is saponified and when it tends to become hard, heat is applied. The castor oil soap product is melted

and gradually heated to a temperature at which vapors begin to come off. The temperature is held at this point so that about 4-9% of the distillate is removed during a period of about 3-5 hours. The resulting product is completely miscible with mineral oil.

In the preparation of greases containing a soluble castor oil soap, the soap is made as outlined above and then, while hot, the mineral oil is stirred into the soap to form a homogeneous mass of the proper consistency and texture.

The following example will illustrate the invention:

| Percent.                                                 |      |    |
|----------------------------------------------------------|------|----|
| Castor oil                                               | 55.9 | 15 |
| Mineral oil (300 viscosity at 100° F. Saybolt Universal) | 39.0 |    |
| Caustic soda (43% solution)                              | 5.1  |    |

The castor oil was charged to a grease kettle adapted to take off a vapor fraction. Stirring was started and aqueous caustic soda slowly added over a period of about two hours. The mixture was converted to a solid white soap. The mixture was heated and at about 400° F. melted. The temperature was raised to about 500° F. when vapors came off. The temperature was maintained at this point for about 3½ hours and about 5% was removed as vapors. The temperature was then dropped to about 350° F. and the mineral oil gradually added, while stirring, over a period of about 5 hours. The temperature was dropped to around 170° F., a small amount of water added to produce an emulsion, and the grease drawn from the kettle.

The product had a smooth texture and a yellow color. It tested as follows:

|                    |          |      |    |
|--------------------|----------|------|----|
| Penetration        | 298      |      |    |
| Melting point, °F. | 241      |      |    |
| Soda soap          | per cent | 21.8 | 40 |
| Free neutral fat   | do       | 37.9 |    |
| Mineral oil        | do       | 41.4 |    |
| Free alkali        | do       | 0.22 |    |
| Water              | do       | 0.50 |    |

The above example merely illustrates one grease within the scope of the invention. It is contemplated that in this type of greases the soap and oil content may vary within a wide range, say from 10-50% of soap, and 50-90% of neutral oils. Also the castor oil may be partially saponified or substantially completely saponified. However, I prefer to use sufficient caustic to saponify 25-75% of the castor oil in which case sufficient excess castor oil is avail-

able to maintain the free alkali at a minimum. It will also be understood that other ingredients may be incorporated into the grease, such as other soaps and oils. The invention is also useful in the preparation of liquid lubricants and in lubricating compositions in which the castor oil ingredient is present only in a relatively small amount.

5 The lubricants made in accordance with the 10 present invention have the advantages that they are relatively stable and maintain their body and consistency at high temperatures.

Obviously many modifications and variations 15 of the invention, as hereinbefore set forth, may be made without departing from the spirit and scope thereof, and therefore only such limitations should be imposed as are indicated in the appended claims.

I claim:

20 1. The method of preparing an oil-soluble castor oil soap product, which comprises forming a mixture of castor oil and castor oil soap, said mixture being normally insoluble in mineral lubricating oils, heating the mixture to a temperature of around 500° F. and maintaining the 25 temperature for sufficient time to vaporize a portion of the mixture in sufficient amount to render the mixture soluble in mineral oil.

2. The method of preparing an oil-soluble castor oil soap, which comprises saponifying the castor oil with an alkali and heating the resultant soap to a temperature sufficiently high to effect substantial dehydration, thereby forming 5 a product normally insoluble in mineral lubricating oil, then further heating the soap to a temperature of around 500° F. and maintaining the latter temperature for sufficient time to distil from the dehydrated soap a fraction in sufficient 10 quantity to render the soap soluble in mineral lubricating oil.

3. The method of preparing an oil-soluble castor oil soap product, which comprises forming a castor oil soap mixture, normally insoluble in mineral lubricating oil, by reacting castor oil with sufficient alkali to effect saponification of the major portion of the castor oil and heating the mixture to a temperature sufficiently high to effect dehydration thereof, then further 20 heating the mixture to a temperature of upwards of 500° F., and maintaining the latter temperature for sufficient time to distil materials which render said mixture insoluble in mineral oil, whereby an undistilled soap product soluble in 25 mineral lubricating oil is formed.

ONEY P. PURYEAR.